

May 13, 1930.

T. M. BANSFIELD

1,758,876

PICTORIAL REPRODUCTION IN PLAQUE

Filed Oct. 24, 1928



## UNITED STATES PATENT OFFICE

THOMAS M. BANSFIELD, OF CHICAGO, ILLINOIS

## PICTORIAL REPRODUCTION IN PLAQUE

Application filed October 24, 1928. Serial No. 314,626.

This invention relates to pictorial reproductions in plaque. The invention has particular reference to the reproduction of works of art in metal, and relates especially to a distinct manner of finishing the surface of the reproduction. The invention is characterized by having the figures of the painting or picture reproduced, embossed or raised in proper proportion and a distinctive feature 10 of the invention resides in silver-plating the surface, and then using a shadowing material such as lampblack or powdered carbon, for example, to fill in the depressions and accentuate the embossed effect of the characters or 15 objects.

Thus, the invention is essentially embodied in a metal plaque having the characters or objects embossed or raised proportionately from the surface in the casting or pressing 20 of the plaque, and the distinctive surface finishing which, as above mentioned, inheres preferably in a precious metal plating by means of which the plaque is rendered much more attractive and also endurable.

25 Other objects will appear hereinafter.

The invention consists in the combinations and arrangements of parts hereinafter described and claimed.

The invention will be best understood by 30 reference to the accompanying drawings forming a part of this specification, and in which:

Fig. 1 is a face or elevational view of a typical plaque of the invention mounted in 35 a frame; and

Fig. 2 is a vertical sectional view through the plaque and frame mounting shown in Fig. 1.

It will be noted that Fig. 2 indicates the 40 rather pronounced raising or embossing of the characters and objects.

In carrying out the invention in order that the figures or objects may be set out in relief, a plaque base is employed which is preferably composed of copper or other endurable 45 malleable metal. The base relief may be prepared either by a casting or mould process.

Referring particularly to Fig. 2 the plaque base 4 is mounted in a suitable frame 5 and 50 held in place by an appropriate backing 6.

As stated, the plaque base is preferably composed of copper or a copper alloy and the silver or precious metal-plating for the surface is indicated at 7. Silver-plating the surface by electro-plating is the preferred 55 method and after the surface has been plated a shadow material such as lampblack or very finely powdered carbon, for example, is spread upon the surface as indicated at 8 in Fig. 2 and fills the depressions and crevices 60 to accentuate the embossing of the objects in the reproduction. After this powdered substance has been spread upon the finished surface of the plaque, as explained, it is brushed off, but in this process the minute grains of 65 the powder adhere to the finished surface of the plaque in the depressions and crevices to produce a shadowing effect which greatly increases the attractiveness of the plaque.

While I have illustrated and described the 70 preferred form of construction for carrying my invention into effect, this is capable of variation and modification without departing from the spirit of the invention. I, therefore, do not wish to be limited to the precise de- 75 tails of construction set forth, but desire to avail myself of such variations and modifications as come within the scope of the appended claims.

Having thus described my invention, what 80 I claim as new and desire to secure by Letters Patent is:

1. The process of making pictorial reproductions in metal plaque form which consists in preparing a base member in embossed relief, having portions raised proportionately to the pictorial reproduction being made, and having depressions formed between the raised portions, plating the surface with a metal coating, covering the plated surface with a 85 powdered substance to fill said depressions, and then brushing the surface to remove surplus powdered material, leaving said material in the depressions to accentuate the relief.

2. The process of making pictorial reproductions in metal plaque form which consists in preparing a base member in embossed relief, having portions raised proportionately to the pictorial reproduction being made, and having depressions formed between the raised 90 95 100

portions, plating the surface with a precious metal, covering the plated surface with a powdered substance to fill said depressions, and then brushing the surface to remove surplus powdered material, leaving said material in the depressions to accentuate the relief.

3. The process of making pictorial reproductions in metal plaque form which consists in forming a base member of malleable metal in embossed relief, having portions raised proportionately to the pictorial reproduction being made, and having depressions formed between said raised portions, electro-plating the surface with a coating of metal, then spreading finely powdered carbon or lampblack upon the surface to fill said depressions, and then brushing off the surplus powdered material but allowing said material to remain in said depressions to accentuate the relief.

4. The process of making pictorial reproductions in metal plaque form which consists in forming a base member of copper or copper alloy in embossed relief, having portions raised proportionately to the pictorial reproduction being made, and having depressions formed between said raised portions, electro-plating the surface with a coating of precious metal, then spreading finely powdered carbon or lampblack upon the surface to fill said depressions, and then brushing off the surplus powdered material but allowing said material to remain in said depressions to accentuate the relief.

35 In testimony whereof I have signed my name to this specification.

THOMAS M. BANSFIELD.

40

45

50

55

60

65